

## UNITED STATES PATENT OFFICE

2,429,648

## METHODS OF PRODUCING ALLOYS LOW IN CARBON

Ivar Rennerfelt and Bo Mikael Sture Kalling,  
Djursholm, SwedenNo Drawing. Application April 8, 1943, Serial No.  
482,890. In Sweden March 11, 1939

5 Claims. (Cl. 75—28)

1

This application is a continuation-in-part of our co-pending application Serial No. 318,894, filed February 14, 1940.

The present invention relates to the treatment of ferro-chrome alloys and has particular reference to the treatment of such alloys in which the ferrous metal content is relatively high, as for example alloys obtainable by the reduction of low grade chrome ores not adapted to be converted to usable ferro-chrome of low carbon content by prior refining treatments.

Heretofore chrome ores having a chrome content of the order of at least 60% to 70% have been considered the only desirable grades usable for the production of ferro-chrome of low carbon content and the production of this material from ore of even this quality involves expensive refining processes which since they are well known in the art, need not be described here in detail. One of the required steps in such refinement is decarbonization of the alloy to reduce the carbon content to an acceptable value, particularly when the alloy is to be used in the production of stainless steel.

A relatively simple and cheap decarburizing process for producing low carbon non-alloyed ferrous metal for melting stock and the like has heretofore been proposed (Rennerfelt U. S. Patent No. 2,170,158) and in the disclosure of that process it has been stated that the process may be employed to decarburize, among other materials, ferro-chrome alloys.

We have, however, discovered that the decarburization of ferro-chrome alloys of the kind now ordinarily produced is not feasible by means of the process disclosed by Rennerfelt, which is based essentially upon treatment in an oxidizing gas atmosphere at high temperature of the metal to be decarburized, with the metal in subdivided or pellet form in order to provide the ratio of surface area to volume of metal required to enable the gas to act effectively. The reason for this is that in such an atmosphere, the chrome, which has a high affinity for oxygen, is rapidly oxidized as well as the carbon. The loss of the valuable alloying element due to such oxidation is alone an undesirable factor. The factor which, however, prevents the successful use of the gaseous oxidizing process to decarburize the usual ferro-chrome alloy is that the oxidized chrome forms an enveloping film of chrome oxide covering the surface of the particle under treatment, and the nature of this oxide is such that it forms in effect a film-like shield which is impervious to the action of the oxidizing gas. As a result, when

2

the usual ferro-chrome alloy is subjected to the above treatment, there is an initial reaction, productive of some decarburization at the surface of the particle, accompanied by the simultaneous formation of chrome oxide film which as it forms progressively slows down and finally acts to substantially stop the reaction. This formation of film acting to substantially stop the reaction occurs sufficiently rapidly to prevent the material lying substantially below the surface of the particle from becoming appreciably decarburized.

We have, however, discovered that the decarburizing of ferro-chrome alloys can successfully be accomplished by gaseous oxidizing methods if the treatments as heretofore attempted are modified either with respect to the nature of the material subjected to the treatment or with respect to the steps of the treatment, or both.

We have found that if the iron content of a ferro-chrome alloy is very substantially increased as compared with the maximum content heretofore considered practically usable, the character of the oxide film formed when the material is subjected to an oxidizing gas atmosphere apparently changes very radically in its nature, particularly with respect to its reaction to the activity of the oxidizing gas. Not only is the content of chromium in the oxide reduced in case of an alloy high in iron content but we believe that the nature of the oxide, which is a complex iron-chrome-oxygen compound, possesses essentially different chemical characteristics from those of a chrome oxide of the kind formed when a high chrome ferro-chrome alloy is subjected to oxidizing treatment.

This difference in the characteristics of the oxide surface film appears to affect the gaseous equilibrium of the oxidizing gases at the surface so that the carbon is the element primarily oxidized and while a certain amount of chrome is oxidized the very much greater velocity of diffusion of the carbon from the interior of the particle to the surface than that of the chrome enables decarburization to be effectively accomplished without undue loss of chrome.

Even more important than this, however, is that when the iron content of the alloy is materially increased as compared with that in the alloys heretofore considered practically usable, the nature of the chrome-iron oxide film changes from the usual hard and impervious nature of a chrome oxide to a pervious nature which permits the oxidizing gases to continue to react with the material being treated.

Consequently, with a high iron content alloy

decarburization can be carried out with gaseous oxidation to an extent enabling the carbon content of the alloy to be brought down to very low values.

We have found that a ferro-chrome alloy having from 20% to 25% chrome, with the remainder mainly iron and carbon, may readily be decarburized in a gaseous oxidizing atmosphere to an extent reducing the carbon content to as little as 0.10% or even lower, if the material is finely subdivided and heated long enough at a temperature preferably within the range of from 1000° C. to 1200° C.

In order to secure the desired results, a high iron content alloy is first provided. This may be done by reducing a suitable mixture of chrome and iron ores with carbon in a furnace, which may be electric or a common blast furnace. The iron required to produce the desired high iron content analysis may also be added in metallic form. Obviously, the extent to which iron will be required to be added will depend upon the quality of the chrome ore employed and in the case of ores of extremely low quality additions of iron (either in the form of ore or as metal) may not be required in order to obtain the high iron content alloy suitable for the decarburizing treatment.

For the small particle size suitable for the gaseous decarburizing treatment, the alloy may advantageously be liquified and then granulated and cooled in water, or it may also be brought to suitable size which is an average particle size of 1.0 to 1.5 millimeters, by crushing. Preferably, particularly if crushing is employed, the carbon content of the initial alloy is relatively high, that is to say, of the order of 3% to 5%.

The temperature at which decarburization is carried out should be as high as practically possible without risk of sintering and consequently sticking of the particles to each other or the furnace wall. Thus the temperature should not materially exceed 1200° C. and a temperature of the order of 1100° C. is more to be preferred.

Decarburization may advantageously be effected by bringing the heated material into contact with a gas mixture containing CO and CO<sub>2</sub> in suitable proportions, preferably, if the atmosphere contains only these gases, in the ratio of approximately 25%-75%. It may be advantageous to oxidize in vacuo or to dilute the CO-CO<sub>2</sub> mixture with other gases such as H<sub>2</sub> or N<sub>2</sub>, in order to obtain the most favorable gaseous equilibrium. However, too high a concentration of nitrogen should be avoided since we have found that this gas may become absorbed in the metal. Hydrogen, however, increases the velocity of the reaction, and may with advantage be supplied to the furnace. In order to supply the quantity of oxygen required to decarburize, without at the same time introducing a supply of nitrogen, it has been found advantageous to introduce steam or water vapor into the reaction zone, the dissociation of which also acting to enrich the H<sub>2</sub> content of the atmosphere. This produces a gas containing H<sub>2</sub>, H<sub>2</sub>O, CO, and CO<sub>2</sub>, and this gas may be burned with air in the cooler zones of the furnace for preheating the charge without risk of absorption of nitrogen into the alloy.

Because of the fact that an oxide film is formed during the reaction, it may in any case be advantageous not to carry the decarburization to the ultimate degree desired in an oxidizing atmosphere, but to finish the process in a reducing

or hydrogen atmosphere. Thus we have found it suitable to decarburize a 20% chrome alloy having a 5% carbon content down to about 0.25% carbon in an oxidizing atmosphere, thereafter treating the material in a hydrogen atmosphere, by which the carbon content may be brought down to 0.05% or less, while at the same time the oxide film is reduced.

As previously noted the ability to successfully decarburize by reaction with a gaseous oxidizing atmosphere is apparently due to the pervious character of the oxide formed at the surface of an alloy high in iron content and to that end the chrome content of the alloy prepared for decarburizing treatment is advantageously not over about 30% and is preferably of the order of 20%-25%. Alloys of higher chrome content are, however, susceptible to gaseous oxidation treatment for decarburizing purposes if the nature of the oxide formed from the higher chrome content alloys is taken into account and the treatment modified accordingly.

Generally speaking, it appears that the higher the chrome content of the alloy, the more the oxide takes on the hard tenacious and impervious qualities of a true chrome oxide. Consequently, if the alloy is relatively high in chrome content the reaction, if not entirely stopped by the oxide film, is retarded to an extent making the process undesirable if not wholly impractical. In such instances the difficulty may, however, be overcome by introducing what may be termed a "washing" step into the process. Assuming a relatively high chrome alloy to be treated, the initial gaseous treatment may be the same as for a low chrome content material. This will result in a progressive slowing down of the reaction due to the formation of relatively less pervious film, the rate at which the reaction is slowed down depending upon the chrome content of the alloy. When this occurs the character of the gaseous atmosphere is altered by the introduction of a film removing or washing agent of suitable nature which may for example be chlorine. Removal of the oxide film by the washing agent permits the decarburizing reaction to be resumed, and, by washing as required, the desired degree of decarburization may be accomplished.

Various forms of furnace may be employed and in many instances it may be found desirable to mechanically agitate the material during the decarburizing treatment, particularly in the case of treatment of high iron content alloys.

What is claimed:

- 55 1. The method of producing low carbon ferro-chrome from a high content chrome ore which consists in preparing in finely divided state an alloy including iron and chromium, reducing said high content chrome ore including the step of adding iron in suitable form to bring the chrome content of the prepared material within the range of substantially from 20% to 30% chrome for subsequent decarburization, and decarburizing said alloy at a temperature below the melting point thereof.
- 60 2. The method of producing low carbon ferro-chrome which consists in preparing in finely divided state an alloy including iron and chromium having a carbon content substantially higher than that desired in the end product, subjecting the resulting material at a temperature below the melting point thereof to decarburization until the decarburization is inhibited by an oxide film, removing said oxide film by the use of
- 65
- 70
- 75

chlorine, and thereafter further decarburizing the allow at below the melting point thereof.

3. The method of producing low carbon ferro-chrome which consists in preparing in finely divided state an alloy including iron and chromium having a carbon content substantially higher than that desired in the end product, subjecting the resulting material at a temperature below the melting point thereof to decarburization until the decarburization is inhibited by an oxide film, removing said oxide film by means of an oxide film removing agent, and thereafter further decarburizing the alloy at below the melting point thereof.

4. The method of producing low carbon ferro-chrome from a high content chrome ore, which consists in preparing in finely divided state an alloy including iron and chromium, reducing said high content chrome ore including the step of adding iron in suitable form to the ore to reduce the percentage of the chrome content of the prepared material to the desired low value for subsequent decarburization, and decarburizing said alloy at a temperature below the melting point thereof to reduce its carbon content.

5. The method of producing low carbon ferro-chrome which consists in utilizing in finely divided

state an alloy including iron and chromium with the chromium content not over approximately 30%, such alloy not forming an objectionable oxide film during decarburization, and in which alloy the carbon content is substantially higher than that desired in the end product, and decarburizing said alloy at a temperature below the melting point thereof to reduce its carbon content.

10

IVAR RENNERFELT.  
BO MIKAEL STURE KALLING.

#### REFERENCES CITED

The following references are of record in the file of this patent:

#### UNITED STATES PATENTS

| Number    | Name       | Date          |
|-----------|------------|---------------|
| 2,170,158 | Rennerfelt | Aug. 22, 1939 |
| 20 96,633 | Thoma      | Nov. 9, 1869  |
| 314,004   | Edwards    | Mar. 17, 1885 |
| 1,086,019 | Bucher     | Feb. 3, 1914  |

#### FOREIGN PATENTS

| 25 Number | Country | Date         |
|-----------|---------|--------------|
| 817,471   | France  | May 24, 1937 |